

# UNITED STATES PATENT OFFICE.

JAMES RAMSEY SPEER, OF TRAPPE, MARYLAND, AND WILLIAM L. FORSTER, OF ROCHESTER, PENNSYLVANIA, ASSIGNEES TO PITTSBURGH IRON & STEEL FOUNDRIES COMPANY, OF MIDLAND, PENNSYLVANIA, A CORPORATION OF PENNSYLVANIA.

## ALLOY OF IRON.

1,071,364.

Specification of Letters Patent.

Patented Aug. 26, 1913.

No Drawing.

Application filed March 18, 1913. Serial No. 755,162.

To all whom it may concern:

Be it known that we, JAMES RAMSEY SPEER and WILLIAM L. FORSTER, citizens of the United States, residing at Trappe, in the county of Talbot, State of Maryland, and at Rochester, in the county of Beaver, State of Pennsylvania, respectively, have invented new and useful Improvements in Alloys of Iron, of which the following is a specification.

Our invention relates to an alloy of iron known as "adamite." The main constituents of our new alloy are iron, silicon, sulfur, phosphorus, manganese, carbon, nickel, and chromium, with or without small quantities of copper, tungsten, and other rare metals which do not materially affect the character of the alloy as hereinafter described.

Our alloy is especially remarkable in that its tensile strength closely approximates that of steel while it has characteristics of cast iron. Tests of bars of our alloy cut from an untreated casting have shown the following:

|    | Transverse breaking load. | Deflection in inches. | Tensile strength in lbs. per sq. in. |
|----|---------------------------|-----------------------|--------------------------------------|
| 30 | 6900 lbs.                 | .12                   | 52,580                               |
|    | 6630 lbs.                 | .11                   | 51,100                               |
|    | 7000 lbs.                 | .10                   | 55,680                               |
|    | 6950 lbs.                 | .11                   | 63,150                               |

In these transverse tests the breaking loads were applied at the center of the bars midway between their end supports, which were ten inches apart. The diameter of each bar was 1.245 inches.

Generically, our invention comprises castings containing the elements and the percentages thereof following: silicon .10% to 2.00%; chromium .5% to 1.50%; nickel .25% to 1.00%; sulfur below .05%; phosphorus below .12%; manganese .45% or less, and total carbon 1.25% to 3.50%. Such castings show remarkable results in tensile and transverse strength, and in wearing and abrasive qualities, and in resistance to the action of heat.

Hereinafter we give various analyses of castings which are specific embodiments of our generic invention, defined in the paragraph next preceding this paragraph.

Analysis of samples of the bars herein-

before referred to showed their composition to be as follows: silicon .70%, sulfur .033%, phosphorus .040%, manganese .25%, total carbon 1.88%, nickel .50%, and chromium .90%.

We have found that in casting various sections the amount of silicon and carbon must be varied in accordance with general foundry practice to get the desired results; and it is for that reason that the maximum and minimum limits which we have given for silicon and total carbon are quite far apart. In fact, we would not limit ourselves to the amount of silicon and carbon mentioned herein in case the castings to be made should have a very enormous section. For example, the variation in the analyses depending on the size of the casting is best shown by the examples following: In the case of a casting 28 inches in diameter, the analysis was:—silicon, .60%; sulfur, .03%; phosphorus, .048%; manganese, .30%; total carbon, 2.13%; nickel, .50%; chromium, 1.05%. The result was a very hard resistant material, requiring the lowest lathe speed and the highest grade of tool steel to dress it.

In the case of a 1 inch or 2 inch tube mill plug, two analyses were as follows: silicon, 1.55%, 1.70%; sulfur, .023%, .023%; phosphorus, .096%, .096%; manganese, .45%, .45%; total carbon, 2.93%, 3.20%; nickel, .43%, .43%; chromium, .85%, .85%. The results obtained in these cases were materials which were hard and resistant to the action of abrasion under heat, and susceptible of being forged. Forging a steel of over 3% carbon is a feat hitherto unknown.

We have found that our alloy wears ten times longer than the best grade of cast iron obtainable for comparison, and in a number of cases its wearing quality has shown even a greater degree of efficiency. Our alloy has a remarkable resistance to abrasion under the action of heat. It has shown an efficiency of from five to ten times that of cast iron where constant wear under the action of heat was the characteristic considered.

We do not deem it proper to designate our alloy "adamite", as either iron or steel, as these words are commonly known to the trade; we believe we have made the discovery of a new composition of metals, which,

in its primary or cast state, resembles cast iron in its action under cutting tools in the lathe, under the acetylene torch, and in its failure to show elasticity or elongation or reduction of area over ordinary cast iron, whereas in its secondary or worked state its ultimate strength, its forging and wearing qualities class it with a steel product.

We have not found it feasible or possible 10 to produce our alloy commercially in a cupola or like furnace. The pneumatic process can be used but at great expense on account of re-carburizing to the extent that is necessary for our alloy. The crucible 15 process may also be used, but its greater cost and smaller units of production make it an inconvenient and costly method of producing even such smaller weight castings of our alloy as the size of crucibles would 20 permit. The air furnace may also be used for making our alloy, but the control of temperature and carbon and silicon in this type of furnace is difficult and rather unsatisfactory for a uniform product. We 25 have found that the regenerative open hearth furnace or the electric furnace is best adapted for producing "adamite". In these furnaces the required control of the temperature at the time of melting and of 30 pouring, which is essential, can be had, which is not possible in a cupola or like furnace. Also the constituent analyses as given for our alloy cannot be obtained from the cupola or like furnace in the case of castings 35 of larger section. In attempting to make our alloy in a cupola the percentages of silicon, sulfur and phosphorus we have found too high to get uniform results. We have found that any such percentages of silicon, 40 sulfur and phosphorus as are contained in the metal, the tests of which were reported in the Iron Age, as above stated, would be destructive to the remarkable results which we have obtained and described herein. In 45 producing our alloy in a regenerative open hearth or electric furnace, the analyses of the product may be figured with exactness in the raw materials; the alloys being combined and used in combination with iron 50 as it occurs in the raw material charge, or as metallic oxids, or as ferro-alloys, or as refined metal, for example, metallic nickel.

We follow the customary and well known 55 method of all steel makers, who use regenerative open hearth furnaces or electric furnaces, in making up our charge of raw materials and as is well known in the art we may use steel scrap in our raw material charge, of the proper analyses to enable us 60 to secure the proper proportion of carbon, silicon. The same result, however, can be obtained by not using any scrap but working the carbon and silicon out of the charge with the addition of ore. After we have 65 introduced our charge in the melting fur-

nace, no chemical action of any considerable importance need necessarily take place provided our raw materials run close to the figured analyses; in other words, if the raw materials run close to the required analyses, our process is a melting one, the getting of sufficient heat to enable us to pour the casting of the size required. If, however, our materials in the raw material charge do not run in analyses as figured, it may be necessary for us to hold a charge in the furnace a sufficient length of time to eliminate elements, as silicon and carbon, which run higher than we have figured them. If the required elements are lower than the figured analyses, we add in the furnace what is lacking to give us metal of our alloy composition, as noted herein. It is understood that the usual loss in melting in furnaces is allowed for and taken care of in the ordinary manner. It is not necessary in all cases to add material which will produce a slag to reduce this oxidation, because a certain amount of slag will naturally be produced from the nature of the materials charged. We desire however, to cover any addition of material necessary to control oxidation. If our alloy is made in a regenerative open hearth furnace it may have either an acid or a basic lining as commonly known in the trade. However, our preference is for the acid-bottom furnace.

It has been claimed that iron castings containing nickel and chromium with a high total carbon content is of value. From our experience we do not attach any importance to the increased carbon contained in such castings, made with the combination of alloys similar to ours; at least, no such results can be obtained in tensile and transverse strengths as we have obtained in our alloy where the control of the carbon is not complete in connection with the control of the silicon, depending upon the size and sections of the castings. It has also been claimed that manganese over .25% in steel metal mixtures containing nickel and chromium is most harmful where hardness and toughness are the special qualities required. From our experience we do not attach any importance to this claim for low manganese in a higher carbon alloy such as ours. Our best results are obtained, as previously stated, by a complete control of the carbon and silicon; the manganese varying in usual limits without any serious effect.

We have found in certain sections of our castings that it is necessary to anneal such castings to preserve their uniform strength and hardness. In this feature our alloy 125 strongly resembles steel. After the metal has been cast as described, we have found that in castings of large section, if they are tumbled out of the molds as promptly as can be done without affecting their solidity, they 130

have a tendency of self-hardening in the air. A similar method to this can be adopted for any class of castings where the wearing service is the essential feature. In the case of castings which are to be forged or dressed for use as tools, we prefer to follow the practice of annealing first, although this is not always essential, then forging and finishing them and finally plunging them into hot water or oil to secure the degree of hardness required. We have found that we can produce an alloy of the two analyses given below, which can be so treated. It can be forged into a lathe tool or drill and properly annealed and hardened. The performance of these tools is the equal of the highest grade of crucible tool steel. The analysis of one sample was: silicon .70%, sulfur .033%, phosphorus .040%, manganese .250%, carbon 1.88%, nickel .50%, chromium .90%. The analysis of another sample was: silicon .60%, sulfur .033%, phosphorus .073%, manganese .22%, carbon 2.26%, nickel .53%, chromium .90%. The tensile strength of the first sample showed 91,220 lbs. per sq. in. without any change in area, elongation, or elastic limit other than would be observed in cast iron. The structure of such material after being forged is similar in every respect to the highest grade of tool steel made in a crucible furnace. The advantage of this method of producing our alloy is obvious for the reason that the manufacturing cost is considerably less than crucible steel, and we are not depending in any way upon any of the rarer and more expensive elements for our results. Our alloy is also particularly adaptable for making drop forgings, of intricate design, where the casting can be made of "adamite" of larger size than the desired finished forging and the finishing can be completed in one set of dies and in one operation; in this way,

greatly reducing the cost of such forgings. Our product is suitable for the greatest variety of uses. It may be used for castings, both large and small, where wear and resistance to heat are important factors. It may also be used for tools, such as hammers, axes, picks, shovels, saws, and in fact, it is particularly adaptable for use generally on account of its dual nature of cast iron and steel. The amount and expense of finishing can be greatly reduced for the reason that "adamite" will, in its primary or cast state, take the form of the article to be manufactured, requiring, in consequence, only a small amount of finishing in its secondary or worked state.

We claim—

1. As a new article of manufacture, an alloy comprising essentially silicon .10% to 2.00%; chromium .5% to 1.50%; nickel .25% to 1.00%; sulfur, not exceeding .05%; phosphorus, not exceeding .12%; manganese, not exceeding .45%, total carbon 1.25% to 3.50%; and iron approximately sufficient to complete the 100%.

2. As a new article of manufacture, an alloy comprising essentially the following elements in substantially the following proportions: silicon .70%, sulfur .033%, phosphorus .04%, manganese .25%, total carbon 1.88%, nickel .50%, chromium .90%, and iron approximately sufficient to complete the 100%.

Signed by the said JAMES RAMSEY SPEER at Midland, Pa., this 11th day of March, A. D. 1913, and by the said WILLIAM L. FORSTER, at Midland, Pa., this 11th day of March, A. D. 1913.

JAMES RAMSEY SPEER.  
WILLIAM L. FORSTER.

Witnesses:

C. BROOKS,  
FRANK B. FOSTER.